

# United States Patent

[19]

Massy et al.

[11] 3,874,848

[45] Apr. 1, 1975

[54] **PROCESS FOR TREATING  
NON-KERATINS MATERIAL WITH A  
POLYTHIOL RESIN AND AN AMINOPLAST  
AND THE PRODUCT OBTAINED**

[75] Inventors: **Derek James Rowland Massy,  
Linton; Kenneth Winterbottom,  
Whittleford, both of England**

[73] Assignee: **Ciba-Geigy AG, Basle, Switzerland**

[22] Filed: **May 16, 1973**

[21] Appl. No.: **360,874**

## Related U.S. Application Data

[63] Continuation of Ser. No. 156,052, June 23, 1971,  
abandoned.

## Foreign Application Priority Data

July 2, 1970 United Kingdom ..... 32240/70

[52] U.S. Cl. .... **8/115.6, 8/116 R, 8/182,  
8/184, 117/139.4, 117/139.5 A**

[51] Int. Cl. .... **D06c 29/00**

[58] **Field of Search..... 8/115.6, 116 R, 128, 127.6,  
8/182, 184; 117/141, 139.4, 139.5 A**

## [56] References Cited

### UNITED STATES PATENTS

3,706,527 12/1972 Dobinson et al. .... **8/115.6 X**  
3,753,649 8/1973 Dobinson et al. .... **8/115.6 X**

*Primary Examiner*—Stephen J. Lechert, Jr.  
*Attorney, Agent, or Firm*—Joseph G. Kolodny; Edward  
McC. Roberts; Prabodh I. Almaula

## [57] ABSTRACT

The present invention relates to a process for improving the mechanical properties of cellulosic fibres. The effects are achieved by impregnating the fibres, especially those treated with an aminoplast, with a resin containing at least two mercaptan groups linked through poly(oxyalkylene) chains to a radical of a polyhydric alcohol.

**19 Claims, No Drawings**

**PROCESS FOR TREATING NON-KERATINS  
MATERIAL WITH A POLYTHIOL RESIN AND AN  
AMINOPLAST AND THE PRODUCT OBTAINED**

This is a continuation of application Ser. No. 156,052, filed on June 23, 1971 now abandoned.

This invention relates to a process for modifying cellulosic materials in fibrous form, and to materials so treated.

It is well known to treat cellulosic materials with amionoplasts. Cellulosic textiles are often treated with these substances to impart dimensional stability, resistance to creasing, or permanent mechanical effects such as pleats and seersucker effects. One drawback is that the tear-strength of the treated textile is often lowered, another is that the treated textile is often harsher. These drawbacks have, to a certain extent, been overcome by incorporating softening agents such as polyethylene emulsions or adducts of ethylene oxide with phenols or amines, but for many purposes these agents are insufficiently effective.

It has now been found that, by the use of certain thi-olterminated poly(oxyalkylene) substances, preferably in conjunction with particular aminoplasts, cellulosic materials having improved properties, in particular textiles having a fuller, softer handle, can be obtained.

Accordingly, the present invention provides a process for modifying cellulosic fibres which comprises

1. treating the fibres, in the absence of keratinous material, with,
    - A. a polythiol having at least two thiol groups per molecule and containing
      - a. radical of a polyhydric alcohol,
      - b. bound to this radical, at least two poly(oxyalkylene) chains,
      - c. bound through oxygen atoms to carbon atoms in the said poly(oxyalkylene) chains, at least two residues selected from the group comprising an acyl residue of a thiol-containing aliphatic carboxylic acid and the residue, after removal of a hydroxyl group, of a thiol-containing aliphatic alcohol,

and, optionally,

  - B. an aminoplast which is free from ethylenic unsaturation, and
  2. curing the polythiol and/or the aminoplast on the fibres.

The present invention further provides cellulosic fibrous materials, in the absence of keratinous material, bearing thereon a polythiol as aforesaid in the cured or still curable state.

If an aminoplast is used, treatment of the fibres with the aminoplast and the polythiol, and curing the polythiol and aminoplast, can take place in any desired sequence. For example, the fibres may be impregnated with a mixture of the aminoplast and the polythiol, and then the aminoplast and/or the polythiol are cured. Or the fibres may be impregnated first with the polythiol and then with the aminoplast, or vice versa, and then the aminoplast and/or polythiol are cured. Or the aminoplast can be cured on the fibres, which are then treated with the polythiol and the polythiol is cured.

Cellulosic fibres which may be subjected to the process of this invention include cotton, regenerated cellulose, including viscose and cuprammonium rayons, jute, linen, hemp, ramie, sisal, paper, and blends of these cellulosic materials with synthetic fibres. The

term cellulosic fibres includes fibres comprised of a substance derived from a cellulose in which some, but not all, of the three available hydroxyl groups per anhydrogluco unit have been chemically modified, e.g. by acylation, etherification, or cyanoethylation. Thus, methyl cellulose and cellulose monoacetate are included but not, for example, cellulose triacetate. The cellulosic materials are preferably textiles, including yarns, threads, woven, non-woven and knitted fabrics, and garments.

Mixtures of two or more cellulosic fibrous materials, and blends with synthetic fibres, may also be treated, but it should be clearly understood that blends of cellulosic fibrous materials with keratinous material are not included within the scope of the present invention.

Polythiols used in the process of this invention preferably contain two, three, or up to six thiol groups per molecule. Especially good results have been obtained with those containing two or three thiol groups per molecule.

Preferred polythiols are those having a molecular weight between 400 and 10,000 particularly those of formula



in which

$m$  is an integer of at least 1 and may have different values in each of the  $p$  and  $(q-1)$  chains.

$n$  is a positive integer of at most 2.

$p$  is a positive integer of at least 2.

$p$  is a positive integer of at least 2,  
 $q$  is a positive integer such that  $(p + q)$  equals at least 3 and at most 7.

each 'alkylene' group contains a chain of at least 2 and at most 6 carbon atoms between consecutive oxygen atoms.

R represents an aliphatic radical containing at least 2 carbon atoms.

and X represents an aliphatic radical containing at least one thiol group.

The oxyalkylene units in individual poly(oxyalkylene) chains may be different. They may be substituted, if desired, by e.g., phenyl or chloromethyl groups,



in which R, 'alkylene',  $m$ ,  $p$ , and  $q$  have the meanings previously assigned, and  $r$  is a positive integer which may be as high as 18 or even 24.

Further preferred are esters of the formula



in which 'alkylene',  $m$ ,  $p$ , and  $q$  have the meanings previously assigned,

*u* is a positive integer of at most 2,  
and R<sup>1</sup> represents an aliphatic radical having at least 15  
2 and at most 6 carbon atoms.

Yet further preferred are esters of formula



and



in which

'alkylene',  $m$ , and  $u$  have the meanings previously assigned, 35

$p_2$  represents 2 or 3,

$p_1$  is zero or 1, such that  $(p_1 + p_2)$  is 2 or 3,

$P_3$  denotes an integer of at least 3 and at most 6, and  $R^2$  represents an aliphatic hydrocarbon radical having at least 3 and at most 6 carbon atoms. 40

Still further preferred are esters bases on based hexane-1,2,5-triol, hexane-1,2,6-triol, ethylene glycol, or propylene glycol, and ethylene oxide and/or propylene oxide, i.e. those of the formulae



30 in which  $m$  and  $u$  have the meanings previously assigned, and  $t$  is an integer of at least 2 and at most 3; and



the polythiol having an average molecular weight between 1000 and 7500, where  $m$  has the meaning previously assigned.

Polythiol esters most preferred for the purposes of the present invention are those obtained from glycerol or propylene glycol, propylene oxide, and thioglycolic acid, i.e. of formula



having a molecular weight within the range 1,000 to 5,000, or even 7,500,

60



and



having a molecular weight within the range 1000 to 7500, where  $m$  has the meaning previously assigned. Such esters are commercially available.

These thiol-terminated poly(alkylene oxide) esters are readily prepared by the reaction of a polyhydric alcohol with an alkylene oxide followed by partial or complete esterification of the terminal hydroxyl groups with a mercaptocarboxylic acid.

Suitable polyhydric alcohols include ethylene glycol, 15 poly(oxyethylene) glycols, propylene glycol, (poly(oxypropylene) glycols, propane-1,3-diol, poly(epichlorohydrin)s, butane-1,2-diol, butane-1,3-diol, butane-1,4-diol, butane-2,3-diol, poly(oxy-1,1-dimethylethylene) glycols, poly(tetrahydrofuran)s, glycerol, 1,1,1-trimethylolethane, 1,1,1-trimethylolpropane, hexane-1,2,5-triol, hexane-1,2,6-triol, pentaerythritol, dipentaerythritol, mannitol, sorbitol, and adducts of allylene oxides with ammonia or amines, such as diethanolamine and tetrakis (N-(2-hydroxyethyl) ethylenediamine. Suitable alkylene oxides include ethylene oxide, propylene oxide, tetrahydrofuran and, less preferably, epichlorohydrin. If desired, the polyhydric alcohol may be treated with one alkylene oxide, say propylene oxide, and then "tipped" with a different alkylene oxide, such as ethylene oxide.

The preferred mercaptocarboxylic acids for the esterification are, as already indicated, thioglycollic acid (2-mercaptopropionic acid) and 2-mercaptopropionic acid, but other mercaptomonocarboxylic acids which may be used include mercaptoundecyclic acid and mercaptostearic acid.

Preferred thiol-terminated poly(alkylene oxides) for use in the invention include those of formula



in which

$R^3$  denotes  $-\text{OH}$ ,  $-(\text{O-alkylene})_u\text{OH}$ ,  $-\text{O.CO.C}_u\text{H}_{2u}\text{SH}$ , or  $-(\text{O-alkylene})_v\text{O.CO.C}_u\text{H}_{2u}\text{SH}$ ,

$R$ , 'alkylene',  $m$ ,  $p$ ,  $q$ , and  $u$  have the meanings previously assigned,

and  $v$  is an integer of at least 1 and may have different values in each of the  $p$  chains.

The oxyalkylene units in the individual poly(oxyalkylene) chains may likewise be different, but are preferably the same, and may be substituted if desired by e.g. phenyl or chloromethyl groups.

Preferred among such ethers are those which are also 60 of formula



in which 'alkylene',  $R^1, m, R^3, p$ , and  $q$  have the meanings previously assigned, and further preferred are those of the formula



10 in which  $R^2$ ,  $R^3$  and  $p_3$  also have the meanings previously assigned.

The particularly preferred ethers are of formula



20 in which  $R^2$ ,  $t$ ,  $m$ , and  $p_3$  have the meanings previously assigned. The ethers in which  $R^3$  denotes  $-\text{OH}$  may be prepared in a known manner by reaction of an alkylene oxide with a polyhydric alcohol, etherification of the hydroxyl groups of the product with epichlorohydrin,

25 and treatment with sodium hydrosulphide to replace the chlorine by a sulphhydryl group ( see U.S. Pat. No. 3,258,495, and United Kingdom Specifications 1,076,725 and 1,144,761). In many cases the average number of thiol groups per molecule is not an integer but, for example, may be 2.6. This is attributable partly to the replacement of the chlorine atoms by the  $-\text{SH}$  group not going to completion, and partly to side-reactions: for example, the chlorohydrin ether obtained by reaction with epichlorohydrin may also react with epichlorohydrin, so forming an ether which contains two replaceable chlorine atoms per hydroxyl group originally present in the polyhydric alcohol.

Ethers of formula



40 in which  $R^2$ ,  $t$ ,  $m$ ,  $v$ , and  $p_3$  have the meanings previously assigned, are likewise particularly preferred. Ethers in which  $R^3$  denotes  $-(\text{O-alkylene})_u\text{OH}$  may be prepared by treating the product which is obtained from epichlorohydrin, the alkylene oxide and the polyhydric alcohol, first with an alkylene oxide, and then with sodium hydrosulphide ( see United Kingdom Specification 1,144,761).

45 The most preferred ethers are those of formula



OH



OH



OH

55 where  $m$  has the meaning previously assigned, especially such ethers having a molecular weight within the range 700 to 3,500 or up to 7500.

The ether-esters in which  $R^3$  denotes  $-\text{O.CO.C}_n\text{H}_{2n}\text{SH}$  or  $-(\text{O-alkylene})_n\text{O.CO.C}_n\text{H}_{2n}\text{SU}$  are obtainable by esterification of the corresponding alcohol with a mercaptocarboxylic acid  $\text{HOOC}_n\text{H}_{2n}\text{SH}$ .

Many of the polythiols which can be used in the invention are insoluble in water but can be applied as aqueous dispersions or emulsions. They may also be applied from organic solvents, for example, lower alkanols such as ethyl alcohol, lower ketones such as ethyl methyl ketone, benzene, and halogenated hydrocarbon solvents, especially chlorinated and/or fluorinated hydrocarbons containing not more than three carbon atoms, such as the dry-cleaning solvents, carbon tetrachloride, trichloroethylene, and perchloroethylene.

The amount of the polythiol to be used depends on the effect desired. When the polythiol is used without an aminoplast, then, for most purposes, from 0.5 to 15 percent by weight calculated on the weight of the material to be treated is preferred. Woven fabrics usually require from 1 to 10 percent by weight of the polythiol, but rather smaller quantities are usually needed on knitted fabrics, say from 1 to 5 percent by weight. The hand, or handle, of the treated material will, of course, depend on the amount of polythiol employed, and by simple experiment the least amount required to give the desired effect may readily be determined. Further, the composition of, and the construction of, fabrics composed of the fibres also influence the amount of polythiol required. When the polythiol is used in conjunction with an aminoplast, the amount of polythiol will be smaller, say from 0.1 to 3 percent by weight calculated on the weight of material to be treated.

The aminoplasts employed contain, per molecule, at least two groups of formula  $-\text{CH}_2\text{OR}^4$  directly attached to an amidic nitrogen atom or atoms, where  $R^4$  denotes a hydrogen atom, an alkyl group of from one to four carbon atoms, or an acetyl group. Examples of such aminoplasts are the IV-hydroxymethyl, N-alkoxymethyl, and N-acetoxyethyl derivatives of following amides and amide-like substances.

I. Urea, thiourea, and the cyclic ureas having the formula



in which

Y denotes either a group of formula



or a divalent group containing from 2 to 4 carbon atoms in the chain, which may be substituted by methyl, methoxy, and hydroxy groups, and which may be interrupted by  $-\text{CO}-$ ,  $-\text{O}-$ , or



where  $R^5$  denotes an alkyl or hydroxyalkyl group containing up to 4 carbon atoms,

and Q denotes oxygen or sulphur,

Examples of such cyclic ureas are ethyleneurea (imidazolidin-2-one), dihydroxythyleneurea (4,5-dihydroimidazolidin-2-one), hydantoin, uron (tetrahydro-oxadiazin-4-one), 1,2-propyleneurea (4-methylimidazolidin-2-one), 1,3-propyleneurea (hexahydro-2H-pyrimid-2-one), hydroxy-

propyleneurea (5-hydroxyhexahydro-2H-pyrimid-2-one), dimethylpropyleneurea (5,5-dimethylhexahydro-2H-pyrimid-2-one), dimethylhydroxypropyleneurea and dimethylmethoxypropyleneurea (i.e. 4-hydroxy- and 4-methoxy-5,5-dimethylhexahydro-2H-pyrimid-2-one), and 5-ethyl- and 5-(2-hydroxyethyl)-triazin-2-one.

II. Carbamates and dicarbamates of aliphatic monohydric and dihydric alcohols containing up to four carbon atoms, e.g. methyl, ethyl, isopropyl, 2-hydroxyethyl, 2-methoxyethyl, 2-hydroxy-n-propyl, and 3-hydroxy-n-propyl carbamates, and ethylene and 1,4-butylene dicarbamates.

III. Melamine and other polyamino-1,3,5-triazines.

If desired, aminoplasts containing both N-hydroxymethyl and N-alkoxymethyl, or N-hydroxymethyl and N-acetoxyethyl groups, may be used, for example, a hexamethylol melamine in which from 1 to 5 of the methylol groups have been so etherified or esterified.

The aminoplast is usually applied as such but, if desired, when a urea-formaldehyde or melamine-formaldehyde product is to be used, it may be formed in situ in a conventional manner from a ureaformaldehyde concentrate or melamine-formaldehyde concentrate and the requisite additional urea or melamine.

The aminoplasts employed are, in general, soluble in water and may be applied from aqueous solution; or they may be applied from aqueous emulsions, from solutions in the dry-cleaning solvents already mentioned, or from solutions in mixtures of water and a suitable co-solvent, such as methanol.

The proportions of the polythiol and the aminoplast can vary widely; usually there will be employed, per thiol group equivalent of the polythiol, from 2 to 50 or even 75, but usually from 5 to 40, N-methylol, N-alkoxymethyl or N-acetoxyethyl group equivalents of the aminoplast.

The desired effects may not be fully obtainable until substantially all the polythiol on the material has cured. At ordinary temperatures this may take from 5 to 10 days or even longer. The curing reaction can, however, be accelerated greatly by the use of a catalyst and generally it is preferred to add the catalyst to the material to be treated at the same time as the polythiol is applied, although it may be added before or afterwards if desired. The curing time can be controlled by selecting an appropriate catalyst and the choice of curing time will depend on the particular application of the process according to the invention.

The catalysts may be bases, siccatives, sulphur, sulphur-containing organic compounds, and free-radical catalysts such as azodi-isobutyronitrile peroxides and hydroperoxides, or combinations of these.

As organic bases there may be used primary or secondary amines such as the lower alkanolamines, e.g. mono- and di-ethanolamine, and lower alkylene polyamines, e.g. ethylenediamine, diethylenetriamine, triethylenetetraamine, tetraethylenepentamine, propane-1,2- and -1,3-diamine, and hexamethylenediamine. As inorganic bases there may be used the water-soluble oxides and hydroxides, e.g. sodium hydroxide, water-soluble, strongly basic salts such as trisodium phosphate, disodium tetraborate, and sodium carbonate, and also ammonia.

Sulphur-containing organic compounds which may be used as catalysts include those in which the sulphur atoms are not exclusively present as mercaptan groups, especially mercaptobenzothiazoles and their derivatives, dithiocarbamates, thiuram sulphides, thioureas, disulphides, alkyl xanthogen sulphides and alkyl xanthates.

Examples of siccatives are calcium, copper, iron, lead, cerium, and cobalt naphthenates.

Examples of suitable peroxides and hydroperoxides are cumene hydroperoxide, tert-butyl hydroperoxide, dicumyl peroxide, dilauryl peroxide, methyl ethyl ketone peroxide, di-isopropyl peroxydicarbonate, and chlorobenzoyl peroxide.

Yet other catalysts are salts of a heavy metal with an acid having an acid strength ( $-\log pK$ ) below 5, or chelates of a heavy metal, including chelates which are also salts. By "heavy metal" is meant one classified as heavy in Lange's Handbook of Chemistry, revised 10th Edition, McGraw-Hill Book Co., at pp. 60-61, that is, a metal of group IB, IIB, IIIB, IVB, VB, VIB, VIIB, or VIII, a metal of group IIIA having an atomic number of at least 13, a metal of group IVA having an atomic number of at least 32, or a metal of group VA having an atomic number of at least 51. Preferably the metal is a member of group IB, IIB, IVB, VB, VIB, VIIB, or VIII, particularly the first series of such metals, i.e. titanium, vanadium, chromium, manganese, nickel, and especially iron, cobalt, and copper. Suitable salt-forming acids are mineral acids, especially hydrochloric, hydrobromic, nitric, sulphuric, phosphorous, and phosphoric acids, and organic acids such as chloroacetic, fumaric, maleic, oxalic, salicylic, and, more especially citric acid. Suitable chelating agents include those in which the chelating atoms are oxygen and/or nitrogen, for example, 1,2- and 1,3-diketones such as acetylacetone, alkylene diamines such as ethylenediamine, and more particularly, ethylenediaminetetraacetic acid.

The amount of catalyst used can vary widely. In general from 0.1 to 20 percent, and usually 1 to 10 percent by weight based on the weight of the polythiol used is required, although much larger quantities can be used.

Curing of the polythiol is also assisted by using elevated temperatures and if especially rapid results are required then temperatures in the range 30° to 180°C may be used. High humidities also tend to accelerate curing in the presence of catalysts. Curing is also promoted by working at a pH in the range 7.5 to 12.

The aminoplast, where one is added, may be cured under the usual conditions, i.e. at room temperature or at elevated temperatures. The mechanism by which the polythiol exerts its effect in conjunction with the aminoplast is not known. It is believed that either the  $-SH$  group of the mercaptan reacts with the N-methylol groups (present as such or formed in situ from esterified or etherified N-methylol groups), or oxidation of

the  $-SH$  groups occurs, molecules of the polythiol being coupled by means of disulphide bridges. The utility of this invention, however, does not depend on the truth of this belief.

5 In many cases it is desirable to use a catalyst for curing the aminoplast. Catalysts which may be used include conventional materials such as latent acid compounds (which may be metal salts), or mixtures thereof, or certain basic substances. Ammonium salts 10 which are latent acids, developing acidity in the mixture on heating, include ammonium chloride, ammonium dihydrogen phosphate, ammonium sulphate and ammonium thiocyanate. These ammonium salts may be used admixed with metal salts which also have a similar 15 catalytic effect. Amine salts may also be used, e.g. 2-amino-2-methylpropanol hydrochloride. Among the suitable latent acid metal salts are zinc nitrate, zinc fluoroborate, zinc chloride, zirconium oxychloride, magnesium chloride, magnesium fluoroborate, and magnesium dihydrogen orthophosphate. These catalysts are generally used at concentrations of 0.3 to 5 percent by weight, calculated on the weight of the fibres.

There may also be used stronger acids such as hydrochloric or sulphuric acids which may be used as an 25 aqueous solution (say, as 4- to 8- normal solutions) or which may be dissolved in a mixture of water and a solvent which is immiscible or partly miscible with water, and also acidic gases. Basic substances which may be used include sodium bicarbonate and sodium carbonate. When strong acid catalysts are used, in liquid or gaseous form, heating may not be necessary. In other cases, it may be necessary to heat the treated material, e.g. at a temperature of from 80° to 200°C for from 30 30 seconds to 10 minutes, and preferably at from 120° to 35 180°C for from 2 to 7 minutes.

The polythiol, and the aminoplast and catalyst if used, can be applied to the material in conventional ways. For example, where fabric is to be treated, they 40 may be padded on, or the material may be immersed in a bath. If garments or garment pieces are to be treated then it is convenient to spray them with the agents, and more convenient still to tumble the garments with the agents dissolved in an organic solvent. For the latter 45 method a dry-cleaning machine using a dry-cleaning solvent is particularly useful.

A crease-resistant finish may be applied to a cellulosic textile fabric by impregnating with the polythiol, an aminoplast and a catalyst for curing the aminoplast, 50 drying the textile, usually in a flat configuration, and then curing at least the aminoplast, normally at a high temperature. Compared to fabric treated with aminoplast only, fabric treated in the above manner is considerably softer and has either substantially improved dry 55 crease-resistance with no further loss in tear strength or substantially improved tear strength with no loss in dry crease-recovery.

A cellulosic textile fabric having good wet crease-recovery properties may be obtained by impregnating 60 the fabric in an aqueous medium with an aminoplast (such as methylolated dihydroxyethylene urea) and a strong acid catalyst (e.g. hydrochloric acid) for curing the aminoplast, keeping the fabric wet and in an uncreased state (e.g. for 16-24 hours), rinsing the fabric 65 if desired, neutralising the catalyst, drying the fabric if necessary, and treating with the polythiol (with an amine or other catalyst if necessary). Material after-treated with the polythiol has much better wet crease-recovery than, and equal tear strength to, fabric treated

with aminoplast alone. Cellulosic textile fabrics having both wet and dry crease-recovery may be obtained by similar treatment, and curing the aminoplast while the fabric is moist. By wet we mean having a water content of more than 20 percent by weight, and by moist we mean having a water content of from 5 to 20 percent by weight, both calculated on the weight of the bone-dry fabric.

A durably pressed cellulosic garment may be made by treating a cellulosic fabric in piece form with the polythiol (say, as an aqueous emulsion or a solution in an organic solvent), an aminoplast, and a catalyst for the aminoplast, and drying the impregnated fabric, fashioning the sensitised fabric into a garment, inserting any requisite creases or pleats and curing the aminoplast at elevated temperature, e.g. in an oven. Compared with garments treated with aminoplast only, the garment is much softer to the touch and has a much better balance of crease-recovery and strength.

under reflux for 16 hours in an atmosphere of nitrogen. Water (20 ml) formed during the reaction was removed as its azeotrope with perchloroethylene. The mixture was worked up as before, to leave 1023 g of the desired bis(thioglycolate), (Thiol B), having a mercaptan content of 0.82 equiv./kg.

### Thiol C

Thiol C denotes a poly (2-hydroxy-3-mercaptopropyl) ether prepared from a glycerol-propylene oxide adduct having an average molecular weight of 4,800, epichlorohydrin, and sodium hydrosulphide. It had a mercaptan content of 0.32 equiv./kg, corresponding to 2.6 SH groups per average molecule.

### Thiols D-L

These Thiols were made in a similar manner to Thiol A. Their compositions are given in the following Table.

| Thiol | Alcohol            | Polyol | Alkylene oxide  | M.W. | Esterifying acid     | Mercaptan Functionality (Theoretical) | Mercaptan content eq./kg |
|-------|--------------------|--------|-----------------|------|----------------------|---------------------------------------|--------------------------|
| D     | Glycerol           |        | Propylene oxide | 3000 | Thioglycollic        | 3                                     | 0.72                     |
| E     | Glycerol           |        | Propylene oxide | 6200 | Thioglycollic        | 3                                     | 0.30                     |
| F     | Glycerol           |        | Propylene oxide | 700  | Thioglycollic        | 3                                     | 2.9                      |
| G     | Glycerol           |        | Propylene oxide | 4000 | Thioglycollic        | 2                                     | 0.41                     |
| H     | Pentaerythritol    |        | Propylene oxide | 2000 | Thioglycollic        | 4                                     | 1.22                     |
| I     | 1,2,6-Hexane-triol |        | Propylene oxide | 1500 | Thioglycollic        | 3                                     | 1.63                     |
| J     | Glycerol           |        | Propylene oxide | 4000 | 2-Mercapto-propionic | 3                                     | 0.6                      |
| K     | Butane-1,4-diol    |        | Tetrahydrofuran | 1000 | Thioglycollic        | 2                                     | 1.66                     |
| L     | Glycerol           |        | Propylene oxide | 1000 | 3-Mercapto-propionic | 3                                     | 2.3                      |

Thiol G is a partial ester.

The compositions used in the process of this invention, viz. those containing a polythiol as aforesaid, as an aqueous dispersion or emulsion, or as a solution in an organic solvent, and optionally a catalyst and an aminoplast, may also contain antisoiling, antistatic, bacteriostatic, rotproofing, flameproofing, and wetting agents. They may also contain water-repellents such as paraffin wax, and fluorescent whitening agents.

The following Examples illustrate the invention. Unless otherwise specified, parts and percentages are by weight. The thiols used were prepared as follows:

### Thiol A

A mixture of 800 g (0.2 g-mol.) of a polyoxypropylene triol having an average molecular weight of 4,000 and made from glycerol and propylene oxide, (Polyol A), 55.2 g (0.6 g-mol.) of thioglycolic acid, 5 g of toluene-p-sulphonic acid, and 350 ml of toluene, was heated to reflux with stirring for 4 hours in an atmosphere of nitrogen. Water (10.8 ml, 0.6 g-mol.) formed during the reaction was removed as its azeotrope with toluene. The mixture was cooled and washed with water, and the organic layer was separated. On removing under vacuum the solvent from the organic layer there remained 793 g (94 percent of the theoretical yield) of the desired tris(thioglycolate), (Thiol A), having a mercaptan content of 0.59 equiv./kg.

### Thiol B

A mixture of polyoxypropylene glycol (1000 g) having an average molecular weight of 2000 (0.5 g-mol.) thioglycolic acid (92 g, 1 g-mol.), toluene-p-sulphonic acid (5 g), and perchloroethylene (750 ml), was heated

under reflux for 16 hours in an atmosphere of nitrogen. Water (20 ml) formed during the reaction was removed as its azeotrope with perchloroethylene. The mixture was worked up as before, to leave 1023 g of the desired bis(thioglycolate), (Thiol B), having a mercaptan content of 0.82 equiv./kg.

### Thiol M

Thiol M was prepared in a similar manner to Thiol C except that a glycerol-propylene oxide adduct having an average molecular weight of 700 was used. It had a mercaptan content of 2.17 eq./kg.

Aqueous emulsions of some thiols were then prepared.

#### Emulsion A

|                     |       |
|---------------------|-------|
| Thiol A             | 500 g |
| Emulsifying agent I | 50 g  |
| water               | 450 g |

The components were mixed at room temperature with a Silverson mixer until a uniform emulsion resulted. "Emulsifying agent I" denotes an adduct of a mixture of  $C_{16}$  and  $C_{18}$  aliphatic primary amines (1 mol.) and ethylene oxide (70 mols).

#### Emulsions B & C

These were prepared in the same manner as Emulsion A, but substituting Thiols B & C for Thiol A.

#### Emulsion D

|                               |       |
|-------------------------------|-------|
| Thiol D                       | 500 g |
| Emulsifying agent I           | 50 g  |
| sodium carboxymethylcellulose | 5 g   |
| water                         | 445 g |

The components were emulsified as before.

## Emulsions E-L

Emulsions E-L were prepared in a similar manner to Emulsion D except that Thiol D was replaced by an equal weight of Thiols E-G, A, G, H, J and K respectively.

Polyol A, used for purposes of comparison, denotes a polyoxypropylene triol having an average molecular weight of 4000, i.e., the polyol used in making Thiol A.

In the following examples measurements of crease angles and tear strengths are recorded: these measurements were carried out on samples which had been conditioned by being kept at 20°C in an atmosphere of 66 percent relative humidity overnight.

## EXAMPLE 1

Samples of a bleached cotton poplin (108 g per square metre) were padded with Liquors 1-4 so that the take-up was 70 percent. The samples were dried for 10 minutes at 70°C on tenter frames to their original dimensions and then the compositions were cured. The curing conditions, and measurements of certain properties of the treated samples, are given in Table I.

Liquors 1-4 had the following compositions:

| Liquor 1                                         |            |  |
|--------------------------------------------------|------------|--|
| Aminoplast A                                     | 60 g/litre |  |
| MgCl <sub>2</sub> .6H <sub>2</sub> O<br>in water | 20 g/litre |  |

Aminoplast A is a co-condensate of a methylated hexamethylol melamine containing 4.5 methoxymethyl groups per molecule and dimethylol ethyleneurea.

## Liquors 2-4

Liquors 2-4 were the same as Liquor 1, but contained in addition 30 g per litre of Emulsions A-C respectively.

In this, and the following Examples, the dry crease angles of the treated samples were measured by the Monsanto method, twelve specimens (six folded warpwise, six folded weftwise) being used in each test, the specimens were creased under a 2 kg load for 3 minutes and allowed to recover, suspended over a wire, for 3 minutes before the crease angles were measured. The values given in the Tables are the average of the six obtained by adding the warpwise value to the corresponding weftwise value and dividing by two. Tear strengths were determined by the Elmendorf method according to TAPPI Standard T 414 n-49. Three samples, each 63 mm × 63 mm, were used, and the tear strengths were measured in the warp direction.

Table 1

| Liquor    | Cure<br>Time<br>(mins) | Cure<br>Temp.<br>(°C) | Handle | Crease<br>angle | Tear<br>strength<br>(g) |
|-----------|------------------------|-----------------------|--------|-----------------|-------------------------|
| Untreated | —                      | —                     | —      | 49°             | 528                     |
| 1         | 3½                     | 160                   | harsh  | 104°            | 224                     |
| 1         | 5                      | 145                   | "      | 99°             | 208                     |
| 2         | 3½                     | 160                   | soft   | 130°            | 240                     |
| 2         | 5                      | 145                   | "      | 114°            | 256                     |
| 3         | 3½                     | 160                   | "      | 115°            | 224                     |
| 3         | 5                      | 145                   | "      | 105°            | 272                     |
| 4         | 3½                     | 160                   | "      | 118°            | 288                     |
| 4         | 5                      | 145                   | "      | 124°            | 320                     |

## EXAMPLE 2

Samples of the bleached cotton poplin used in Example 1 were padded with Liquor 1 so that the take-up was 70 percent, and dried for 10 minutes at 70°C on tenter frames to their original dimensions. The samples were heated for 5 minutes at 145°C to cure the aminoplast. Next, some of these samples were padded with a 0.7 percent solution of a thiol in perchloroethylene, the pick-up of the thiol being 1 percent, and then they were dried as before and heated for 3½ minutes at 160°C. The crease angle and tear strengths were measured and they are shown in Table II.

Table II

| Treated with       | Crease angle | Tear strength (g) |
|--------------------|--------------|-------------------|
| Untreated          | 49°          | 528               |
| Liquor 1 only      | 99°          | 208               |
| Liquor 1 + Thiol A | 123°         | 288               |
| Liquor 1 + Thiol B | 129°         | 304               |
| Liquor 1 + Thiol C | 130°         | 272               |

## EXAMPLE 3

Poplin samples were padded with a 0.7 percent solution of the thiol in perchloroethylene to 1 percent pick-up of the thiol. The samples were dried for 10 minutes at 70°C on tenter frames, heated for 3½ minutes at 160°C, then treated with Liquor 1 to 70 percent pick-up. The samples were dried in the same manner as before, and cured for 5 minutes at 145°C. Measurements of the tear strength and crease angle are given in Table III.

Table III

| Treated with       | Crease angle | Tear strength (g) |
|--------------------|--------------|-------------------|
| Untreated          | 49°          | 528               |
| Liquor 1 only      | 99°          | 208               |
| Liquor 1 + Thiol A | 119°         | 228               |
| Liquor 1 + Thiol B | 116°         | 320               |
| Liquor 1 + Thiol C | 131°         | 352               |

## EXAMPLE 4

In order to ascertain the machine-washability of cotton poplin treated in accordance with the present invention, samples were padded to 70 percent pick-up with Liquors 1 and 2. After curing, the handle of the material was noted, and the crease angle and tear strength were measured. The samples were then washed three times, with intermediate tumble drying, in an English Electric Reversomatic washing machine set on programme 1 (90°C wash) using an aqueous solution containing 2 g/litre soap and 0.8 g/litre soda ash. The crease angle and tear strength were again measured: the results are given in Table IV.

Table IV

| Liquor | Cure<br>(mins) | Time<br>(°C) | Handle<br>Original | Handle<br>Washed | Crease angle<br>Original | Crease angle<br>Washed | Tear strength (g)<br>Original | Tear strength (g)<br>Washed |
|--------|----------------|--------------|--------------------|------------------|--------------------------|------------------------|-------------------------------|-----------------------------|
| 1      | 5              | 140          | harsh              | soft             | 92°                      | 73°                    | 240                           | 256                         |
| 2      | 5              | 140          | soft,<br>silky     | soft,<br>silky   | 116°                     | 82°                    | 320                           | 256                         |
| 2      | 3½             | 160          | soft,<br>silky     | soft,<br>silky   | 124°                     | 97°                    | 256                           | 272                         |

## EXAMPLE 5

Aqueous liquors 5 and 6 were prepared containing the following ingredients, expressed in grams per litre of water:

|                                      | Liquor 5 | Liquor 6 |
|--------------------------------------|----------|----------|
| Aminoplast A                         | 60       | 60       |
| MgCl <sub>2</sub> .6H <sub>2</sub> O | 20       | 20       |
| Emulsion A                           | 30       | 60       |

Samples of bleached cotton poplin were padded with the above liquors, and also, for comparative purposes, with Liquor 1, so that the uptake was 70 percent. The samples were dried for 10 minutes at 60°C on tenter frames, then cured for 3½ minutes at 160°C. The crease angles and tear strengths were measured, the samples were then washed three times as described in Example 4, and the tear strengths and crease angles were measured again. Table V shows the results obtained.

Table V

| Liquor | Crease<br>angle | Original<br>Tear<br>strength<br>(g) | Crease<br>angle | Washed<br>Tear<br>strength<br>(g) |
|--------|-----------------|-------------------------------------|-----------------|-----------------------------------|
| 1      | 103°            | 204                                 | 93°             | 236                               |
| 5      | 114°            | 288                                 | 97°             | 340                               |
| 6      | 117°            | 304                                 | 97°             | 352                               |

## EXAMPLE 6

In order to compare the effects of the compositions containing an aminoplast and a polythiol with compositions containing an aminoplast and a conventional softening agent (Softening Agent A) samples of a cotton poplin were treated to 64 percent uptake with the following aqueous liquors:

| Liquor                               | 7   | 8   | 9   | 10  | 11  |
|--------------------------------------|-----|-----|-----|-----|-----|
| Emulsion A                           | —   | 10  | 30  | —   | —   |
| Softening Agent A                    | —   | —   | —   | 10  | 30  |
| MgCl <sub>2</sub> .6H <sub>2</sub> O | 15  | 15  | 15  | 15  | 15  |
| Aminoplast B                         | 150 | 150 | 150 | 150 | 150 |

These figures refer to grams per litre.

Aminoplast B is a 50 percent aqueous solution containing equimolar amounts of the pentamethyl ether of hexamethylol melamine and bis(N-hydroxymethyl) ethyleneurea.

Softening Agent A is a commercially-available product sold for use with aminoplasts.

The samples were dried at 110°C for 1 minute and cured at 150°C for 5 minutes. They were then stored at room temperature. After 1 day, some of the samples were washed in a Hoovermatic washing machine for 30 minutes at 95°C with a solution containing soap flakes (5 g per litre) and sodium carbonate (2 g per litre), and then tested. The remaining samples were tested after 5 days' storage at room temperature.

The results are given in Table VI.

Table VI

| Liquor | Crease<br>angle | Original<br>Tear<br>strength<br>(g) | Crease<br>angle | Washed<br>Tear<br>strength<br>(g) |
|--------|-----------------|-------------------------------------|-----------------|-----------------------------------|
| 7      | 98°             | 467                                 | 95°             | 490                               |
| 8      | 112°            | 518                                 | 96°             | 522                               |
| 9      | 125°            | 616                                 | 110°            | 539                               |
| 10     | 98°             | 549                                 | 95°             | 553                               |
| 11     | 102°            | 616                                 | 97°             | 568                               |

From this Table it may be seen that, by using the thiol, a greatly improved crease angle is obtained for a given tear strength, compared to that obtained using the conventional softening agent.

## EXAMPLE 7

Bleached cotton poplin was padded with a solution of Thiol A in perchloroethylene to 1 percent pick-up of the thiol. The samples were dried for 10 minutes at 60°C and kept at room temperature for 24 hours. They were then treated with an aqueous solution containing an aminoplast and 4 g per litre of ammonium sulphate to 70 percent uptake of solution, dried for 10 minutes at 60°C, and cured for 3½ minutes at 160°C. The crease angles and tear strengths were measured, and are reported in Table VII. Comparative figures for poplin which had not been treated with Thiol A are also given.

Table VII

| Aminoplast                     | Conc. of solution<br>(g/litre) | Crease angle | Tear strength<br>(g) |
|--------------------------------|--------------------------------|--------------|----------------------|
| Treated with Thiol Resin A     |                                |              |                      |
| C                              | 120                            | 80°          | 320                  |
| D                              | 100                            | 83°          | 332                  |
| E                              | 90                             | 86°          | 236                  |
| Not treated with Thiol Resin A |                                |              |                      |
| C                              | 120                            | 68°          | 320                  |
| D                              | 100                            | 73°          | 256                  |
| E                              | 90                             | 72°          | 212                  |

Aminoplast C is a 50 percent aqueous solution of bis(N-hydroxymethyl) dihydroxyethyleneurea.

Aminoplast D is a 75 percent aqueous solution of a methylated methylolmelamine, containing on average three N-methoxymethyl and two N-hydroxymethyl groups per molecule.

Aminoplast E is the pentamethyl ether of hexamethylolmelamine.

#### EXAMPLE 8

Bleached cotton poplin was padded to 70 percent uptake with the following aqueous liquors: (concentration in g per litre)

| Liquor                       | 12  | 13  | 14  | 15  |
|------------------------------|-----|-----|-----|-----|
| Emulsion A                   | 30  | 30  | —   | —   |
| Aminoplast C                 | 120 | —   | 120 | —   |
| Aminoplast D                 | —   | 100 | —   | 100 |
| $(\text{NH}_4)_2\text{SO}_4$ | 4   | 4   | 4   | 4   |

The samples were dried for 10 minutes at 60°C, then cured for 3½ minutes at 160°C. The crease angles and tear strengths were measured, and the results are given in Table VIII.

Table VIII

| Liquor    | Crease angle | Tear strength (g) |
|-----------|--------------|-------------------|
| 12        | 81°          | 332               |
| 13        | 86°          | 316               |
| 14        | 71°          | 228               |
| 15        | 73°          | 256               |
| Untreated | 39°          | 496               |

#### EXAMPLE 9

Bleached cotton poplin was padded to 70 percent uptake with Liquors 14 and 15 as described in Example 8, or with an aqueous liquor (Liquor 16) containing 90 g per litre of Aminoplast E and 4 g per litre of ammonium sulphate, dried for 10 minutes at 60°C, and cured for 3½ minutes at 160°C. Some samples were then treated with a solution of Thiol A in perchloroethylene to give 1 percent pick-up of the thiol. After being dried for 10 minutes at 60°C, the samples were cured for 24 hours at room temperature, and the crease angles and tear strengths were measured, the results being reported in Table IX.

Table IX

| Liquor                          | Crease angle | Tear strength (g) |
|---------------------------------|--------------|-------------------|
| <u>Treated with Thiol A</u>     |              |                   |
| 14                              | 81°          | 476               |
| 15                              | 84°          | 336               |
| 16                              | 87°          | 324               |
| <u>Not treated with Thiol A</u> |              |                   |
| 14                              | 68°          | 320               |
| 15                              | 73°          | 256               |
| 16                              | 72°          | 212               |
| Untreated                       | 39°          | 496               |

#### EXAMPLE 10

An impregnation liquor, comprising 0.2 ml of Emulsion H, 0.2 ml of a 1 percent aqueous solution of monoethanolamine, and 199.6 ml of water, was heated to

60°C and a 10 g hank of scoured cellulose diacetate continuous filament yarn was immersed in the liquor, which was kept at 60°C for 30 minutes, the yarn being moved continuously in the liquor. The hank was removed, spun in a spin dryer, and dried at 70°C. Comparison with untreated yarn showed that a pleasing softening effect had been imparted to the yarn treated in accordance with the process of this invention.

#### EXAMPLE 11

Samples of a bleached cotton poplin (108 g per sq. metre) were padded with Liquors 17-21 so that the uptake was 70 percent. The compositions of the liquors, expressed in grams per litre of water, were as follows:

15

| Liquor                                    | 17  | 18  | 19  | 20  | 21  | 22  |
|-------------------------------------------|-----|-----|-----|-----|-----|-----|
| Aminoplast B                              | 120 | 120 | 120 | 120 | 120 | 120 |
| $\text{MgCl}_2 \cdot 6\text{H}_2\text{O}$ | 18  | 18  | 18  | 18  | 18  | 18  |
| Emulsion H                                | —   | 20  | —   | —   | —   | —   |
| Emulsion D                                | —   | —   | 20  | —   | —   | —   |
| Emulsion E                                | —   | —   | —   | 20  | —   | —   |
| Emulsion F                                | —   | —   | —   | —   | 20  | —   |
| Emulsion I                                | —   | —   | —   | —   | —   | 20  |

The samples were dried for 10 minutes at 70°C on tenter frames to their original dimensions and then cured by heating at 160°C for 3½ minutes. The crease angles and tear strengths of the patterns were measured. The samples were washed 5 times in an English Electric Reversomatic washing machine set on programme 2 (60°C wash) using an aqueous solution containing 2g/l soap and 0.8g/l soda ash, and then tumble-dried. The crease angle and tear strength were again measured: the results are given in Table X.

TABLE X

| Liquor    | Handle                 | Crease angle° |        | Tear strength(g) |        |
|-----------|------------------------|---------------|--------|------------------|--------|
|           |                        | Original      | Washed | Original         | Washed |
| 17        | Harsher than untreated | 92°           | 86°    | 416              | 288    |
| 18        | Soft silky             | 110°          | 94°    | 360              | 348    |
| 19        | Soft silky             | 103°          | 84°    | 388              | 356    |
| 20        | Soft silky             | 112°          | 97°    | 356              | 320    |
| 21        | Soft                   | 102°          | 97°    | 308              | 288    |
| 22        | Waxy                   | 117°          | 100°   | 360              | 372    |
| Untreated | Soft                   | 40°           | 53°    | 920              | 700    |

Tests also showed that the thiol did not interfere with the non-chlorine retentive properties of the resin.

#### EXAMPLE 12

Samples of a bleached cotton poplin (tear strength 792g) were padded with Liquor 1 to 70 percent expression, dried on tenter frames to their original dimensions, and cured by heating for 3½ minutes at 160°C.

Next, some of the samples were padded with a 1.45 percent solution of the Thiol or Polyol A in trichloroethylene to 138 percent pick-up. The trichloroethylene solutions also contained 0.029 percent of diethyltriamine as curing catalyst. The patterns were dried at 70°C on tenter frames to their original dimensions and were then allowed to cure at room temperature for 1 week. The crease angle and tear strength were measured and are recorded in Table XI.

TABLE XI

| Treated with        | Crease angle | Tear strength (g) |
|---------------------|--------------|-------------------|
| Untreated           | 46°          | 792               |
| Liquor I only       | 108°         | 210               |
| Liquor I + Thiol A  | 121°         | 252               |
| Liquor I + Thiol G  | 124°         | 304               |
| Liquor I + Polyol A | 106°         | 312               |

This example illustrates that treatment with Polyol A improves only the tear strength whereas that with the thiols improves both the crease angle and the tear strength.

## EXAMPLE 13

Cotton poplin samples were padded with 1.45 percent solution of Thiol A in trichloroethylene to 138 percent pick-up. In some cases the solutions also contained curing catalysts. The patterns were dried at 70°C to their original dimensions on tenter frames and they were then kept at room temperature for 1 week to allow the thiol to cure. The samples were then treated with Liquor I to 70 percent pick-up, dried at 70°C to their original dimensions, and finally cured by heating for 3½ minutes at 160°C. Some samples were washed three times as described in Example 11. Crease angles and tear strength measurements of the treated patterns are recorded in Table XII.

TABLE XII

| Treated with       | % catalyst<br>(on weight of<br>cotton)        | Crease angle  |        | Tear strength (g) |        |
|--------------------|-----------------------------------------------|---------------|--------|-------------------|--------|
|                    |                                               | Un-<br>washed | Washed | Un-<br>washed     | washed |
| Untreated          | —                                             | 46°           | —      | 792               | —      |
| Liquor I only      | —                                             | 108°          | 98     | 210               | 204    |
| Thiol A + Liquor I | —                                             | 121°          | 110    | 268               | 328    |
| Thiol A + Liquor I | 0.1% Copper<br>naphthalene(8%Cu)              | 132°          | 117    | 208               | 268    |
| Thiol A + Liquor I | 0.2% Diisopropyl<br>xanthogen disul-<br>phide | 128°          | 118    | 248               | 280    |

## EXAMPLE 14

A 50:50 cotton-polyester plain weave fabric was padded with one of Liquors 23-25 to 70 percent pick-up, dried at its original dimensions on tenter frames at 60°C, and finally heated for 10 minutes at 170°C. The crease angles and tear strength were measured and are recorded in Table XIII, as are the compositions of the liquors.

TABLE XIII

| Liquor                                     | Untreated | 23   | 24   | 25   |
|--------------------------------------------|-----------|------|------|------|
| Aminoplast C (g/l)                         | —         | 150  | 150  | 150  |
| MgCl <sub>2</sub> ·6H <sub>2</sub> O (g/l) | —         | 20   | 20   | 20   |
| Emulsion G (g/l)                           | —         | —    | 30   | —    |
| Emulsion H (g/l)                           | —         | —    | —    | 30   |
| Crease angle °                             | 94        | 117  | 122  | 128  |
| Tear strength (g)                          | 1344      | 1320 | 1376 | 1368 |

## EXAMPLE 15

Samples of the bleached cotton poplin used in Example 11 were padded with liquor I to 70 percent expression, dried on tenter frames to their original dimensions, and heated for 3½ minutes at 160°C to cure the

10

5

## 20

aminoplast. Next, some of these samples were padded with a 1.27 percent solution of a thiol and 0.0254 percent of diethylenetriamine in trichloroethylene, the pick-up of the thiol being 2 percent. They were dried as before, and left at room temperature for 4 days. The crease angles and tear strength were measured, as shown in Table XIV.

TABLE XIV

| Treated with       | Crease angle ° | Tear strength (g) |
|--------------------|----------------|-------------------|
| Untreated          | 42             | 916               |
| Liquor I only      | 102            | 316               |
| Liquor I + Thiol A | 120            | 320               |
| Liquor I + Thiol H | 113            | 296               |
| Liquor I + Thiol I | 115            | 292               |
| Liquor I + Thiol J | 126            | 304               |
| Liquor I + Thiol K | 125            | 356               |
| Liquor I + Thiol L | 123            | 272               |
| Liquor I + Thiol M | 114            | 268               |

20

25

## EXAMPLE 16

Poplin samples were padded with a 1.46 percent solution of the thiol or Polyol A in trichloroethylene to 2 percent pick-up of thiol or Polyol A. The samples were dried for 10 minutes at 70°C at their original dimensions on tenter frames. They were then treated with Liquor I to 70 percent expression, dried as before, and cured for 3½ minutes at 160°C. Some samples were

25

25

washed three times by the procedure described in Example II. The crease angles and tear strengths were measured and the results are recorded in Table XV.

TABLE XV

| Treated with        | Crease angle ° |        | Tear strength (g) |        |
|---------------------|----------------|--------|-------------------|--------|
|                     | Un-<br>washed  | Washed | Un-<br>washed     | Washed |
| Untreated           | 44             | —      | 864               | —      |
| Liquor I only       | 101            | 95     | 264               | 244    |
| Thiol A + Liquor I  | 121            | 103    | 316               | 308    |
| Thiol G + Liquor I  | 116            | 103    | 356               | 320    |
| Polyol A + Liquor I | 99             | 89     | 312               | 260    |

60

65

## EXAMPLE 17

Emulsions H and J to L were applied to 10g pieces of scoured cellulose diacetate by the following procedure. Samples of each of the emulsions were first diluted 100 times with water and treatment liquors were then prepared by taking 100 g/l of each of the diluted emulsions and adjusting the pH to 4.0 with acetic acid. The fabrics were treated at a liquor ratio of 20:1 for 30 minutes at 60°C. In some cases hydrogen peroxide sufficient to provide a concentration of 1 volume was





below 5, and chelates of heavy metals.

10. The process of claim 1, which comprises treating the cellulosic fibres with the polythiol at a temperature in the range 30° to 180°C.

11. The process of claim 1, which comprises treating the cellulosic fibres with the polythiol in the form of a solution in an organic medium or in the form of an aqueous dispersion, solution, or emulsion.

12. Hydroxyl-containing cellulosic fibrous materials, free from keratinous material, bearing thereon a cured coating from 0.5 to 15 percent by weight of a polythiol resin and an aminoplast free from ethylenic unsaturation, said polythiol resin having up to six thiol groups per molecule and a molecular weight between about 400 and about 10,000, the polythiol having the formula:



in which

$m$  is a positive integer of at least 1,

$n$  is zero or 1,

$p$  is a positive integer of at least 2 and at most 6,

$q$  is zero or a positive integer of four or less, selected

so that  $(p+q)$  equals at least 2 and at most 6,

each alkylene group contains a chain of at least 2 and at most 6 carbon atoms between consecutive oxygen atoms,

$R$  is an aliphatic radical containing at least 2 carbon atoms, and

$X$  is an aliphatic radical containing at least one thiol group.

13. The cellulosic fibrous material of claim 12, wherein the polythiol is the polythiol defined in claim 10 2.

14. The cellulosic fibrous material of claim 12, wherein the polythiol is the polythiol defined in claim 10 3.

15. The cellulosic fibrous material of claim 12, 15 wherein the polythiol is the polythiol defined in claim 4.

16. The cellulosic fibrous material of claim 12, wherein the polythiol is the polythiol defined in claim 5.

20 17. The cellulosic fibrous material of claim 12, wherein the polythiol is the polythiol defined in claim 6.

18. The cellulosic fibrous material of claim 12, 25 wherein the polythiol is the polythiol defined in claim 7.

19. The cellulosic fibrous material of claim 12, bearing thereon (A) the polythiol and (B) an aminoplast providing from 2 to 75 equivalents of a group selected from the class consisting of N-methylol, N-30 alkoxymethyl, and N-acetoxymethyl groups per thiol group equivalent of said polythiol.

\* \* \* \* \*

35

40

45

50

55

60

65